

84-11

Patented Jan. 11, 1938

2,105,070

## UNITED STATES PATENT OFFICE

2,105,070

## MAGNETIC CORE

Adolph F. Bandur, Berwyn, Ill., assignor to Western Electric Company, Incorporated, New York, N. Y., a corporation of New York

No Drawing. Application February 16, 1934,  
Serial No. 711,552

7 Claims. (Cl. 175—21)

This invention relates to magnetic cores made from finely divided and insulated magnetic particles, and methods for making such cores.

Objects of the invention are to provide cores 5 made of finely divided magnetic particles having high permeabilities and low energy losses and efficient methods of making such cores.

In accordance with one embodiment of the invention, finely divided magnetic material such 10 as finely divided particles of nickel iron alloy are mixed with talc and annealed after which an insulating coating of a metallic hydroxide, sodium silicate and a finely divided refractory metallic silicate is applied and cores formed of the insulated parts.

In carrying out the present invention, the magnetic material is preferably prepared from brittle alloys containing various percentages of nickel and iron. These alloys may be prepared as fully 20 described in the patent to C. P. Beath and H. M. E. Heinicke, No. 1,669,649, issued May 15, 1928.

An alloy thus prepared is rolled while hot into relatively thin slabs and quenched to produce a fine crystalline structure, which is very desirable 25 since the disintegration of the material takes place at the crystal boundaries and consequently the smaller the size of the crystals, the finer the dust which can be produced from the finished product. The magnetic alloy thus 30 received in slab form is reduced to a finely divided form or dust, in any well known manner, as for example, in a hammer mill or other suitable reducing apparatus and subsequently pulverized in an attrition mill.

The dust from the attrition mill is sifted and 35 passed through a 300 mesh sieve. In the case where the magnetic material in the core is a magnetic alloy including nickel and iron it has been found desirable to subject the magnetic 40 particles to a heat treatment at a high temperature to remove the strains introduced in the magnetic material by the grinding operation which tends to impair the magnetic properties of the magnetic alloy in the core. The temperature 45 of this heat treatment should be from 1500° to 1600° F. or higher. However, when the magnetic particles are heated to this temperature they tend to sinter to such an extent that further grinding is required which would again set 50 up strains therein. In order to avoid this difficulty a quantity of finely pulverized magnesium silicate or talc is roasted at a temperature in the neighborhood of 1600° F. This roasting seems to further disintegrate the finely pulverized particles and drives the moisture therefrom. The

magnetic particles are then mixed with approximately .30 percent by weight of the roasted talc and the mixture is annealed at a temperature from 1500° to 1600° F. During this process it appears that the fine particles of talc are imbedded 5 and firmly adhere to the surface of the magnetic particles so as to substantially prevent sintering during the annealing operation. Any slight cohesion between the particles may be readily broken up by a light grinding of the material 10 which is not sufficient to impair the magnetic properties of the particles.

The particles are then insulated with an insulating composition comprising .066 percent magnesium hydroxide (milk of magnesia), .32 15 percent sodium silicate, and .93 percent talc by weight of the magnetic material. This insulation is preferably applied in several coatings. For the first coating a solution is made of about 15 percent of water, .021 percent magnesium hydroxide and .11 percent of sodium silicate. Since a quantity of talc has already been added to the magnetic particles to prevent sintering in the heat treating operation, no talc is added to this solution. The magnetic particles are thoroughly mixed with this solution after which the coated particles are heated to a temperature of 275° to 300° F. to evaporate the water and form an initial set in the insulating material so that it will not be redissolved in the application of 20 subsequent coatings. The second coating is applied by forming a solution of about 13 percent water, .015 percent of magnesium hydroxide, .07 percent of sodium silicate, and .21 percent of talc. The particles are then again heated to dry and 25 set the coating and two additional coatings are applied in the same manner, making a total of four coatings in which approximately .066 percent of magnesium hydroxide, .32 percent of sodium silicate, and .93 percent of talc by weight 30 of the magnetic material, are used. The percentages are based on the weight of the solids or non-volatile constituents of the ingredients, and the amount of insulating material may be varied in accordance with the fineness of the magnetic 35 particles to be insulated.

After the dust has been insulated as described, the magnetic material is formed into cores by subjecting it to a pressure in the neighborhood of 200,000 pounds per square inch. During the application of this pressure the magnetic particles are again subjected to strains which impair the magnetic properties thereof and therefore the cores are again subjected to an annealing heat treatment by heating the cores preferably in a 40

hydrogen atmosphere to a temperature from 1,000° to 1,200° F. In this heat treatment the insulating material also appears to be fully cured.

While it is not desired to be limited to any particular theory, it appears that the sodium silicate in the presence of magnesium hydroxide is converted in the several heat treatments to extremely fine particles, which are much smaller than they would be in the absence of the magnesium hydroxide. The magnesium hydroxide appears to be converted into very fine particles of magnesium oxide. Magnetic particles which pass through a 300 mesh sieve have an average cross sectional dimension about 45 microns or smaller. The talc which is a refractory metallic silicate may have a cross sectional dimension from 2 to 4 microns. In binding the particles of talc together to form an insulating film over the magnetic particles, the sodium silicate appears to form the chief binder and the magnesium oxide being much finer fills in the interstices to form a dense film which will not be disrupted under the high pressure used in forming the core. It has been found that voltages as high as 100 volts may be applied to opposite sides of a core insulated in this manner without breaking down the insulation.

Other metallic hydrates such as bismuth, aluminum, zinc and cadmium hydrates may be used in place of magnesium hydrate. It is also possible to use magnesium sulphate which, due to the presence of the sodium silicate, will be converted to magnesium hydrate and thus produce a similar result. The sodium silicate employed should have preferably a high silicate to soda ratio; preferably a ratio of about 1.6 to 3.0 part silicate to one part soda.

The invention has been described particularly in connection with talc as the refractory metallic silicate. Other refractory metallic silicates such as aluminum silicate or a mixture of aluminum and magnesium silicates may be used. It is also possible to use other alkali metal silicates for the sodium silicate such as for instance potassium silicate, although in the preferred form of the invention sodium silicate is used.

The insulating material described above is particularly useful in insulating very fine magnetic particles. On account of the thin and tenacious film which is formed over the particles, the amount of insulating material used constitutes only a small fraction by weight of the core, which results in a high permeability of the core and the effectiveness of the insulation maintains the eddy current losses in the core at a low value.

What is claimed is:

1. A method of making a magnetic body which comprises applying to finely divided magnetic

particles an insulating coating of a finely divided refractory metallic silicate, magnesium hydroxide and sodium silicate, and heat treating the coating to cure the insulation.

2. A method of making a magnetic body which comprises applying to finely divided magnetic particles an insulating coating of magnesium silicate, magnesium hydroxide and sodium silicate, and heat treating the coating to cure the insulation. 10

3. A method of making a magnetic body which comprises applying to finely divided magnetic particles an insulating coating of finely divided refractory insulating material, magnesium hydroxide and an alkali metal silicate, and heat 15 treating the coating to cure the insulation.

4. A method of making a magnetic body of finely divided magnetic particles which comprises mixing finely divided magnesium silicate with the particles to prevent sintering, annealing the 20 particles, applying an aqueous solution of magnesium hydroxide and sodium silicate to the particles, evaporating the solution to dryness to form an insulating coating on the particles, applying a second aqueous solution of magnesium hydroxide, sodium silicate, and magnesium silicate to the 25 particles, evaporating the solution to dryness, forming a core of the insulated particles, and heating the core.

5. A method of making a magnetic body of 30 finely divided magnetic particles which comprises applying an insulating coating of substantially .066 percent magnesium hydroxide, .32 percent of sodium silicate, and .93 percent of talc, forming cores of the particles, and heat treating the core. 35

6. A method of making a magnetic body of finely divided magnetic particles which comprises adding .3 percent of talc to the particles to prevent sintering, annealing the particles at a temperature in the neighborhood of 1600° F., adding 40 an aqueous solution of .021 percent magnesium hydroxide, .11 percent of sodium silicate, evaporating the solution to dryness, adding a second aqueous solution .015 percent magnesium hydroxide, .07 percent sodium silicate, and .21 percent of talc, evaporating the solution to dryness, adding two additional solutions similar to the second solution and evaporating each of said solutions to dryness, compressing the particles into a core and heat treating the core at a high temperature to 50 improve the magnetic characteristics of the magnetic material therein.

7. A magnetic structure comprising particles of magnetic material separated by insulation comprising the end products of a heat treated mixture 55 of magnesium hydroxide, an alkali metal silicate and a filler.

ADOLPH F. BANDUR.